

Sept. 25, 1951

A. BRENNER  
INSTRUMENT FOR USE IN DETERMINING THE STRESS  
IN AN ELECTRODEPOSIT

2,568,713

Filed April 6, 1949

2 Sheets-Sheet 1

*Fig. 1.*



*Fig. 2.*



INVENTOR  
ABNER BRENNER

BY  
Ray B. Hackley, Jr.  
ATTORNEY

Sept. 25, 1951

A. BRENNER  
INSTRUMENT FOR USE IN DETERMINING THE STRESS  
IN AN ELECTRODEPOSIT

2,568,713

Filed April 6, 1949

2 Sheets-Sheet 2

*Fig. 3.*



*Fig. 4.*

INVENTOR  
ABNER BRENNER  
BY  
Ray C. Hachley Jr.  
ATTORNEY

## UNITED STATES PATENT OFFICE

2,568,713

INSTRUMENT FOR USE IN DETERMINING  
THE STRESS IN AN ELECTRODEPOSITAbner Brenner, Chevy Chase, Md., assignor to  
the United States of America as represented  
by the Secretary of Commerce

Application April 6, 1949, Serial No. 85,922

4 Claims. (Cl. 73—150)

(Granted under the act of March 3, 1883, as  
amended April 30, 1928; 370 O. G. 757)

1

The invention described herein may be manufactured and used by or for the Government of the United States for governmental purposes without the payment to me of any royalty thereon in accordance with the provisions of the act of April 30, 1928 (ch. 460, 45 Stat. L. 467).

My invention relates to a novel apparatus for measuring stress in the electrodeposits by means of the deformation of a helix accompanying the electroplating of said helix with the same or different metal; and particularly to an apparatus which visually registers an increase in deformation during the deposition of the coating. An essential element of my apparatus is a metal helix coated on one cylindrical surface with a suitable varnish which inhibits the electrodeposition of metal upon said surface, while the opposite surface is clean and suitable for receiving an electrodeposited coating.

The electrodeposition of metal on only one cylindrical surface of the metal helix is accompanied by a progressively increasing deformation of the helix which produces a change in the radius of curvature of the helix, and my apparatus is designed to multiply this change and to visually register this movement by an indicating pointer pivoted over a graduated dial face.

In the accompanying drawings which illustrate a preferred form of my invention:

Figure 1 is an axial section of my apparatus.

Figure 2 is a side elevation of a helix used in my apparatus.

Figure 3 is a plan of a pinion, segmental gear, and calibrated disc which serve to magnify the distortion of my helix during an electroplating operation.

Figure 4 is a section on the line 4—4 of Figure 1. In these drawings:

A metallic helix 11 (Figure 2) is coated on the inner cylindrical surface with a suitable varnish which serves to prevent the electrodeposition of metal upon said coated surface. Preferably, this helix is formed by winding a strip of base metal around a cylindrical mandrel annealing the helix, and then removing the helix from the mandrel. The annealed helix is then stretched to leave a spiral gap 12 between successive windings.

A suspending framework 13 comprises a suspending rod 14 having a terminal suspending hook 15 and an offset portion 16, a split clamping collar 17 provided with a suitable clamping screw 18, a shouldered sleeve 19, a second sleeve 20 adapted to fit around the sleeve 19 and to be releasably clamped thereto by a knurled clamping bolt 21.

A shouldered insulating sleeve 22 fits the sec-

ond sleeve 20 while my helix 11 is adapted to telescopically fit over the sleeve 22 and to be detachably secured thereto by a clamping sleeve 23 provided with a bolt 24 which also serves to electrically connect my helix 11 with an insulated conducting wire 25.

To the shouldered sleeve 19 there is bolted a circular plate 26 provided with an aperture for a rod 27 which extends downwardly through the sleeve 19 and helix 11. The rod 27 is suspended from the plate 26 by a supporting sleeve 28 to which it is releasably clamped by a set screw 29. The rod 27 is provided with a boss 30 which arrests upward movement of the rod. To the sleeve 28 is fastened an arm 31 having a terminal segmental gear 32, which meshes with a pinion 33 mounted in adjustable bearings 34. To the pinion 33 is rigidly secured a pointer 35 which is adapted to move over a scale 36 on the plate 26. A centrally apertured insulating plug 37 is adapted to be clamped to the rod 27 by a set screw 38 and is provided with one or more fluid passages 39. A second clamping sleeve 40 provided with a clamping bolt 41 serves to transmit motion from my helix 11 through the plug 37, rod 27, and gear 32 to the pinion 33, and the attached pointer 35. The bearings 34 are mounted in a suitable U-shaped support 42 which is riveted or otherwise fastened to the plate 26. The pointer 35 is provided with a counterbalancing weight 43.

The radii of the segmental gear 32 and the pinion 33 are so proportioned as to give a tenfold magnification of the angular displacement of the rod 27. The sleeve 19 does not make electrical contact with the helix 11 while the clamps 23 and 40 attach the helix 11 to the remainder of the apparatus. These clamps also serve as electrical guards which give a very uniform current distribution over the active surface of the helix 11. Loosening the clamping bolt 29 permits sliding the rod 27 within the sleeve 28, while loosening the knurled bolt 21 permits adjusting shouldered sleeve with respect to other elements of the framework 13.

By relative rotation of the sleeve 20 with respect to the sleeve 19, the pointer 35 may be set at any desired graduation on the dial of the plate 26 and clamped by the bolt 21.

The entire assembly is suspended by the hook 15 within a tank (not shown) containing a suitable plating solution, the level of which is somewhere on the upper clamp 23. By electrically connecting the positive lead from a suitable source of direct current to the anode, and the negative lead to the conducting wire 25, my ap-

paratus is ready to start plating on the helix 11. Since the top of the helix 11 is firmly secured to the suspending framework 13, the bottom only of the helix 11 is free to turn as the plating proceeds, which motion is transmitted through the 5 rod 27 and multiplying gearing to the pointer 35.

Between successive tests only the helix and attaching clamps need to be disconnected from the remainder of the assembled apparatus. After the weight and/or thickness of the coating has been determined the electrodeposit may be stripped from the helix by a suitable chemical solvent.

The plate 26 and the entire registering mechanism may be enclosed in a protective transparent case (not shown).

If coatings of the same thickness are deposited upon the helix, the deflection of the pointer can be taken as a relative measure of the stress existing in the coatings. In some studies of stress in deposits, only the relative value of stress was determined, but it is preferable to state the stress in absolute values in order that the work of different investigators can be compared.

In order to calculate the stress in the deposit from the deflection of the pointer, one must also know the thickness of the coating and the force constant and dimensions of the helix. The constant "K" of the helix is determined by applying a known torque to the helix and noting the deflection of the pointer. The torque is most easily applied by suspending a known weight from the arm of the gear segment, via a pulley and thread.

$$K = \frac{\text{weight (in lb.)} \times \text{distance to pivot (inches)}}{\text{degrees deflection}}$$

$$\text{Stress in coating (lb/in.}^2\text{)} = \frac{2KD}{ptd}$$

K is the constant for the helix as above determined.

p is the pitch of the spiral (inches).

t is the thickness of the strip composing the helix (inches).

d is the thickness of the electrodeposit (inches).

D is the deflection of the pointer in degrees.

The pitch of the helix is measured with a rule. The thickness of the helix strip is measured with a micrometer. The thickness of the electrodeposit is calculated from the weight of coating deposited upon the helix.

The calculation of the stress is simplified by first determining the deflection constant of the helix, that is, the torque required to cause a deflection of one degree. This can be done by attaching a thread to the arm 31 near the gear 32 and passing it over a removable pulley, then with the helix clamped with the pointer at a selected point of the dial, weights are attached to the string and the deflections of the pointer 35 noted. An initial load of 10 to 20 g. may be attached to the string and then as weights are added, recording the increased deflections. By measuring the distance from the axis of the torque rod to the point of attachment of the string on the arm 31 and using the recorded load in grams, a deflection constant may be calculated which shows the relation of the bending movement of the helix to the degrees of deflection.

My apparatus provides a means for investigating the variations in stresses due to variations in the conditions of deposition and to differences in the thickness of the deposits and differences in the grain size of the coatings. Prior to my invention, many authors have discussed the in-

5  
jurious deformations due to stresses which may result in visual failures such as the peeling, blistering or cracking of the deposited coating, which failures render the base metal more susceptible to corrosion.

10  
My apparatus provides a means for registering stress deformations in a coating while it is being deposited and thereby aids in production control and in the improvement of the quality of the plating on articles. It is rugged, easily operated, self-contained, and comparatively inexpensive.

15  
It should be understood that the present disclosure is for the purpose of illustration only, and that the invention includes all modifications and equivalents which fall within the scope of the appended claims.

What I claim is:

20  
1. An instrument for measuring the stress in an electrodeposit, which comprises a metallic helix having on one cylindrical surface a deposit-inhibiting film, on the other a clean surface for receiving an electrodeposit, a suspending framework, a clamping sleeve provided with a suitable electrical terminal for detachably securing said helix to said framework, a rod rotatably mounted in the axis of said framework, a segmental gear secured to the upper end of said rod, a pinion with a pointer supported by said framework and meshing with said gear, an insulating plug clamped to the lower end of said rod, and a second helix clamping sleeve for compressing the lower end of the helix against said plug for transmitting torque due to a deformation of said helix 25 through said plug and said rod to said pointer.

30  
2. An instrument for indicating stress in an electrodeposit during the course of the deposition thereon, comprising a metallic helix having on one cylindrical surface only a deposit-inhibiting film, an electrical terminal at one end of said helix, a suspending framework, means for detachably suspending said helix from said framework, a rod rotatably mounted in the axis of said framework, a segmental gear secured to the upper end of said rod and non-rotatably connected therewith, a pinion supported by said framework and meshing with said gear, and means for transmitting torque to said rod from the lower end of said helix.

35  
3. An instrument for use in determining the stress in an electrodeposit which comprises a metallic helix having on one cylindrical surface only a deposit-inhibiting film, a suitable suspending framework, a clamping sleeve provided with an electrical terminal for detachably suspending said helix from said framework, a rod rotatably mounted in the axis of said framework, a segmental gear secured to the upper end of said rod, a pinion with a rigidly connected pointer supported by said framework and meshing with said gear, an insulating plug clamped to the lower end of said rod, a second helix clamping sleeve for compressing the lower end of the helix against said plug, whereby torque due to any deformation of said helix will be transmitted through said plug and said rod to said pointer.

40  
4. An instrument for use in determining the stress in an electrodeposit during the deposition of a metallic coating on a metal base, comprising a metallic helix having one deposit-receiving cylindrical surface and an opposite surface protected by a deposit-inhibiting film, a helix clamping sleeve provided with an electric terminal, a suspending framework provided with a depending tubular portion, an insulating sleeve on said

tubular portion against which said helix is clamped by said clamping sleeve, a lower insulating plug within the helix provided with a longitudinal aperture for a rod, a lower clamping sleeve for compressing said helix against said plug, a torque transmitting rod within said sleeve non-rotatably connected with said plug, a revoluble motion multiplying means operatively coupled with said torque-transmitting rod, and an indicator for registering said multiplied motion.

ABNER BRENNER.

## REFERENCES CITED

The following references are of record in the file of this patent:

## UNITED STATES PATENTS

| Number    | Name  | Date         |
|-----------|-------|--------------|
| 2,117,287 | Bloch | May 17, 1938 |